

# United States Patent [19]

Bliss et al.

[11] 3,768,997

[45] Oct. 30, 1973

[54] **PROCESS FOR PRODUCING LOW CARBON SILICOMANGANESE**

[75] Inventors: **Norman G. Bliss; Robert T. Wright,**  
both of Kingston, Tenn.

[73] Assignee: **The Mead Corporation, Dayton,**  
Ohio

[22] Filed: **May 22, 1972**

[21] Appl. No.: **255,777**

[52] U.S. Cl. .... **75/10 R, 75/129**

[51] Int. Cl. .... **C22d 7/06**

[58] Field of Search .... **75/10-13, 129, 130, 133.5**

[56] **References Cited**

UNITED STATES PATENTS

|           |         |              |       |         |
|-----------|---------|--------------|-------|---------|
| 3,704,114 | 11/1972 | Wilson       | ..... | 75/10 R |
| 3,431,103 | 3/1969  | Querengasser | ..... | 75/11   |
| 3,149,962 | 9/1964  | Mennenoh     | ..... | 75/11   |
| 2,010,230 | 8/1935  | Gustafsson   | ..... | 75/11   |
| 3,666,438 | 5/1972  | Madronic     | ..... | 75/11   |

3,329,497 7/1967 Deadrick ..... 75/133.5  
3,393,068 7/1968 Robiette ..... 75/133.5

Primary Examiner—L. Dewayne Rutledge

Assistant Examiner—Peter D. Rosenberg

Attorney—Hugh P. Carter et al.

[57]

## ABSTRACT

Low carbon siliconmanganese produced by introducing into a slag free, submerged arc electric furnace charge materials comprising a mixture of gravel, ferromanganese fines, low alloy steel, coal, coke and wood chips in proportions to obtain an alloy composition of about 50 to 65 percent manganese, 20 to 31 percent silicon, 0.05 to 0.80 percent carbon, 0.10 to 0.20 percent phosphorus, a maximum of about 0.05 percent sulfur and the balance essentially iron. An electric current is passed through the submerged electrodes of the furnace to obtain carbonaceous reduction of the charged materials and molten metal is removed periodically adjacent the bottom of the furnace.

12 Claims, No Drawings

## PROCESS FOR PRODUCING LOW CARBON SILICOMANGANESE

### BACKGROUND OF THE INVENTION

This invention relates to a process for producing low carbon siliconmanganese and more particularly to a process which provides a more economical utilization of ferromanganese fines by producing low carbon siliconmanganese adapted for use in controlling carbon in the manufacture of medium carbon ferromanganese, and for use as a low carbon deoxidizing agent for the production of steel.

As is well known in the art to which our invention relates, the disposal of fines produced in the production of ferromanganese is a very difficult problem. Heretofore, it has been the usual practice to remelt the fines. This not only consumes considerable time and energy, but also results in the formation of additional fines.

### BRIEF SUMMARY OF THE INVENTION

In accordance with our invention, we produce low carbon siliconmanganese by introducing into a slag free, submerged arc electric furnace charge materials comprising a mixture of gravel, ferromanganese fines, low alloy steel, coal, coke and wood chips. The components of the mixture are proportioned to obtain an alloy composition of about 50 to 65 percent manganese, 20 to 31 percent silicon, 0.05 to 0.80 percent carbon, 0.10 to 0.20 percent phosphorus, a maximum of about 0.05 percent sulfur and the balance essentially iron. An electric current is passed through the electrodes of the furnace while submerged in the charge materials to bring about carbonaceous reduction of the charged materials. The molten metal alloy is removed periodically adjacent the bottom of the furnace.

### DETAILED DESCRIPTION

In carrying out our process for producing low carbon siliconmanganese, we introduce into a slag free, submerged arc electric furnace charge materials comprising a mixture of gravel, ferromanganese fines, low alloy steel, coal, coke and wood chips. The furnace is thoroughly cleaned whereby all slag is removed therefrom prior to introducing the charge materials. No slag should be left in the furnace due to the fact that a slagless operation is desired so as to eliminate subsequent separation of slag from the product.

The ferromanganese fines employed in our process contain about 65 to 82 percent manganese, 1.0 to 7.5 percent carbon, 0.05 to 3.00 percent silicon, 6 to 14 percent iron and 0.15 to 0.35 percent phosphorus. The ferromanganese fines are sized from 2 inches down.

The gravel employed in our charge materials contains about 95 to 99.5 percent silicon dioxide. The low alloy steel employed contains about 90 to 99.5 percent iron, 0.1 to 2.0 percent manganese and less than 0.05 percent phosphorus. The coal employed in the charge materials contains about 65 to 80 percent dry fixed carbon while the coke employed contains about 75 to 95 percent dry fixed carbon. The wood chips employed in our charge materials contains about 3 to 20 percent natural fixed carbon and are employed to provide burden porosity and to control electrical resistivity of the furnace. The addition of wood chips increases resistivity. Preferably, the low alloy steel is in the form of steel turnings, which, in addition to iron, contain about 0.1 to 2.0 percent manganese and less than 0.05 percent

phosphorus. The ratio of manganese to iron in the charge materials is maintained at 2.6 to 1 or greater.

The charge materials are introduced into the slag free, submerged arc electric furnace initially to fill substantially one half of the furnace, with the electrodes buried in the charge materials current is passed through the electrodes as the remainder of the furnace is filled with the charge materials. Thereafter, the charged materials are introduced continuously as the materials move downwardly to thus maintain the furnace substantially full at all times. The first removal of the molten metal alloy takes place approximately three hours after the current is first passed through the electrodes. The molten metal alloy is then removed every 2 hours.

In actual practice, we have carried out our improved process in a 25 foot shell diameter, 12,000 KVA, three phase submerged arc electric furnace having three electrodes 35 inches in diameter and a crucible approximately 18 feet in diameter and 7 1/2 feet deep. The electrical load employed on this furnace ranges from approximately 9,000 to 11,000 kilowatts at 120 to 200 volts. Since approximately 21 megawatt-hours of energy is consumed in this furnace in two hours, the molten metal alloy is removed from the furnace at the end of each interval in which approximately 21 megawatt-hours of energy have been consumed by the furnace.

To produce our low carbon siliconmanganese, the charge materials are proportioned to obtain an alloy composition of about 50 to 65 percent manganese, 20 to 31 percent silicon, 0.05 to 0.80 percent carbon, 0.10 to 0.20 percent phosphorus, a maximum of about 0.05 percent sulfur and the balance essentially iron.

As an example, the following charge mixture has been found to be satisfactory in every respect to produce an alloy product containing 52.25 percent manganese, 26.29 percent silicon, 0.20 percent carbon, 0.16 percent phosphorus, 0.02 percent sulfur and the balance essentially iron.

### EXAMPLE

#### FURNACE CHARGE MATERIALS

|         |                                   |
|---------|-----------------------------------|
| 500 lb. | Gravel (8.33 parts)               |
| 620 lb. | Standard FeMn Fines (10.33 parts) |
| 80 lb.  | Scrap Steel Turnings (1.33 parts) |
| 230 lb. | Coal (1.83 parts)                 |
| 60 lb.  | Coke (1 part)                     |
| 300 lb. | Wood Chips (5 parts)              |

Analysis of charge materials was as follows

#### GRAVEL

Size 2 1/2" x 1/8"

|                                |        |
|--------------------------------|--------|
| SiO <sub>2</sub>               | 98.46% |
| Al <sub>2</sub> O <sub>3</sub> | 0.59%  |
| Fe <sub>2</sub> O <sub>3</sub> | 0.42%  |
| MgO                            | 0.01%  |
| CaO                            | 0.05%  |

#### STANDARD FERROMANGANESE FINES

Sized 2" x D

|    |    |        |
|----|----|--------|
| 60 | Mn | 73.20% |
|    | Fe | 11.10% |
|    | C  | 6.50%  |
|    | Si | 1.10%  |
|    | P  | 0.17%  |

#### LOW ALLOY STEEL IN FORM OF SCRAP STEEL TURNINGS

|    |        |
|----|--------|
| Fe | 97.85% |
| Mn | 0.48%  |
| Cr | .17%   |

|                   | 0.17%  |
|-------------------|--------|
| <b>COAL</b>       |        |
| Size 2" x 3/8"    |        |
| Volatiles         | 18.60% |
| Ash               | 6.10%  |
| Fixed Carbon      | 71.80% |
| Moisture          | 3.5%   |
| <b>COKE</b>       |        |
| Size 1" x 1/8"    |        |
| Volatiles         | 3.09%  |
| Ash               | 12.93% |
| Fixed Carbon      | 83.97% |
| <b>WOOD CHIPS</b> |        |
| Volatiles         | 85.05% |
| Ash               | 2.20%  |
| Fixed Carbon      | 12.75% |
| Moisture          | 40.40% |

The electric furnace was operated as described hereinabove for a period of 28 2/3 days. During this time 1,452.2 net tons of alloy were produced consuming approximately 2.02 KWH per pound of alloy. 78 percent of the manganese in the charged materials was recovered in the alloy.

From the foregoing, it will be seen that we have devised an improved process for producing low carbon silicomanganese. By forming silicomanganese from standard ferromanganese fines, we not only eliminate the problem of disposing of such fines but at the same time provide an economical process for utilizing such fines in producing low carbon silicomanganese which is particularly adapted for carbon control in forming other alloys.

We wish it to be understood that we do not desire to be limited to the precise examples, proportions or embodiments herein disclosed for obvious modifications will occur to persons skilled in the art.

What we claim is:

1. The process for producing low carbon silicomanganese comprising the steps of:
  - a. introducing into a slag free, submerged arc, electric furnace charge materials comprising a mixture of approximately the following parts by weight: 8.33 parts gravel, 10.33 parts ferromanganese fines, 1.83 parts coal, one part coke, 5 parts wood chips and 1.33 parts low alloy steel containing about 90 to 95 percent iron, 0.1 to 2.0 percent manganese and less than 0.05 phosphorus,
  - b. passing an electric current through the electrodes of said furnace while the electrodes are submerged in said charged materials in an amount to obtain carbonaceous reduction of said charged materials and an alloy composition of about 50 to 65 percent manganese, 20 to 31 percent silicon, .05 to .80% carbon, 0.10 to 0.20 percent phosphorus, a maximum of about .05% sulfur and the balance essen-
2. The process for producing low carbon silicomanganese as defined in claim 1 in which said gravel contains about 95 to 99.5 percent silicon dioxide.
3. The process for producing low carbon silicomanganese as defined in claim 1 in which said ferromanganese fines contains about 65 to 82 percent manganese, 1.0 to 7.5 percent carbon, 0.05 to 3.00 percent silicon, 6 to 14 percent iron and 0.10 to 0.35 percent phosphorus.
4. The process for producing low carbon silicomanganese as defined in claim 1 in which said ferromanganese fines range in size from 2 inches down.
5. The process for producing low carbon silicomanganese as defined in claim 1 in which said coal contains about 65 to 80 percent dry fixed carbon.
6. The process for producing low carbon silicomanganese as defined in claim 1 in which said coke contains about 75 to 95 percent dry fixed carbon.
7. The process for producing low carbon silicomanganese as defined in claim 1 in which said wood chips contain about 3 to 20 percent natural fixed carbon.
8. The process for producing low carbon silicomanganese as defined in claim 1 in which said molten metal is removed at the end of each interval in which approximately 21 megawatt-hours of energy have been consumed by said furnace.
9. The process for producing low carbon silicomanganese as defined in claim 1 in which the charge materials are initially introduced into said furnace to fill substantially one half of said furnace at the time current is passed through said electrodes and then the remainder of said furnace is filled with said charge materials and said charge materials are introduced continuously thereafter as current is passing through said electrodes.
10. The process for producing low carbon silicomanganese as defined in claim 1 in which the first removal of molten metal takes place approximately 3 hours after said current is first passed through said electrodes and then molten metal is removed every 2 hours thereafter.
11. The process for producing low carbon silicomanganese as defined in claim 1 in which the ratio of manganese to iron in said charge materials is at least 2.6 to 1.
12. The process for producing low carbon silicomanganese as defined in claim 1 in which the electrical load employed on a 25 foot shell diameter, 12,000 KVA, 3 phase submerged arc electric furnace having 3 electrodes 35 inches in diameter and a crucible approximately 18 feet in diameter and 7 1/2 feet deep ranges from approximately 9,000 to 11,000 kilowatts at 120 to 200 volts.

tially iron, and

c. removing molten metal periodically adjacent the bottom of said furnace.

5. The process for producing low carbon silicomanganese as defined in claim 1 in which said gravel contains about 95 to 99.5 percent silicon dioxide.

10. The process for producing low carbon silicomanganese as defined in claim 1 in which said ferromanganese fines contains about 65 to 82 percent manganese, 1.0 to 7.5 percent carbon, 0.05 to 3.00 percent silicon, 6 to 14 percent iron and 0.10 to 0.35 percent phosphorus.

15. The process for producing low carbon silicomanganese as defined in claim 1 in which said ferromanganese fines range in size from 2 inches down.

20. The process for producing low carbon silicomanganese as defined in claim 1 in which said coke contains about 75 to 95 percent dry fixed carbon.

25. The process for producing low carbon silicomanganese as defined in claim 1 in which said wood chips contain about 3 to 20 percent natural fixed carbon.

30. The process for producing low carbon silicomanganese as defined in claim 1 in which said molten metal is removed at the end of each interval in which approximately 21 megawatt-hours of energy have been consumed by said furnace.

35. The process for producing low carbon silicomanganese as defined in claim 1 in which the charge materials are initially introduced into said furnace to fill substantially one half of said furnace at the time current is passed through said electrodes and then the remainder of said furnace is filled with said charge materials and said charge materials are introduced continuously thereafter as current is passing through said electrodes.

40. The process for producing low carbon silicomanganese as defined in claim 1 in which the first removal of molten metal takes place approximately 3 hours after said current is first passed through said electrodes and then molten metal is removed every 2 hours thereafter.

45. The process for producing low carbon silicomanganese as defined in claim 1 in which the ratio of manganese to iron in said charge materials is at least 2.6 to 1.

50. The process for producing low carbon silicomanganese as defined in claim 1 in which the electrical load employed on a 25 foot shell diameter, 12,000 KVA, 3 phase submerged arc electric furnace having 3 electrodes 35 inches in diameter and a crucible approximately 18 feet in diameter and 7 1/2 feet deep ranges from approximately 9,000 to 11,000 kilowatts at 120 to 200 volts.

\* \* \* \* \*